

## UNITED STATES PATENT OFFICE

2,048,594

## ELECTRODEPOSITING METALS

Charles Joseph Brockman, Athens, Ga.

No Drawing. Application January 21, 1935,  
Serial No. 2,837

12 Claims. (Cl. 204—1)

This invention relates to the art of electro-depositing metals. More particularly it concerns the electrodeposition of one metal upon another in instances where because of the relative characteristics of the metals, particularly their electromotive potentials, it is difficult to plate satisfactorily by ordinary methods from the usual highly ionized solutions.

In such instances it quite frequently happens that if the metal upon which the deposit is to be made, be immersed in the plating bath, it will immediately receive a coating of the metal to be deposited without any outside current being applied. Unfortunately, the coating so formed is nearly always of a spongy, poorly adherent nature and serves only to prevent the adherence of the deposit later to be made.

In order to avoid the formation of this poorly adherent deposit a number of modifications of the basic plating procedures have been tried and some are now in use. In general these modifications fall into two classes. Either the object to be plated is first covered with an intermediate or "strike" coating of a metal that will form an adherent deposit on the object and the final coating deposited on the surface so formed, or the plating conditions are so modified that the metal with which it is desired to plate will not form a spongy deposit of the kind mentioned.

Various changes in plating conditions have been tried, including the starting of the deposition at a rate so rapid that the spongy, poorly adherent deposit cannot form. It has not been possible in all cases, however, to start the plating rapidly enough to do this without seriously impairing the quality of the metal deposited. Hence, the industry has in many instances turned to other changes in plating conditions for the solution to the problem and many new plating baths have been developed for electro-depositing the metals without the initial spontaneous formation of the poorly adherent coating.

Among the baths used for the purpose of eliminating the spongy coating, the cyanide baths are probably the most common. Copper can be directly plated upon iron or steel from an alkaline copper cyanide solution, although the cathode efficiency is relatively poor, the bath is extremely poisonous and the current density must be carefully controlled. Usually a thin "strike" coating of copper is applied by the use of a cyanide solution and the plating then finished in a copper sulfate bath. Other metals may be similarly deposited by the use of cyanide baths upon cathodes on which they will not ordinarily form an

adherent deposit. However, the disadvantages of plating from a cyanide solution are much the same regardless of the metal plated.

Because of these disadvantages at least several additional types of baths have been developed and tried under various conditions. Of these mention may here be made of two, the tartrate bath and the "oxalato" bath, both used for plating copper on steel or iron. A tartrate bath suggested by Brown and Mathers, J. Phys. Chem. 10 39-51 10 (1906) has the following formula:

|                           |            |
|---------------------------|------------|
| Copper sulfate            | 60 grams   |
| Sodium hydroxide          | 50 grams   |
| Sodium potassium tartrate | 159 grams  |
| Water                     | 1 liter 15 |

The "oxalato" bath was suggested by Fink and Wong, Trans. Electrochem. Soc. 63 Preprint 9 (1933). It is also aqueous and has the formula:

|                                                    |                |
|----------------------------------------------------|----------------|
| Copper oxalato (Disodium diaquodioxalato cuproate) | 20             |
| $Na_2[Cu(C_2O_4)_2 \cdot (H_2O)_2]$                | 20 grams/liter |
| Sodium sulfate                                     | 15 grams/liter |
| Boric acid                                         | 20 grams/liter |

The authors tell us that their baths obviate many of the difficulties experienced with the cyanide type of bath.

Nevertheless, experiments indicate that the current efficiency, quality of the deposit and other features of the methods using these baths are still subject to improvement. Hence, it is the purpose of the present invention to provide a new method involving the use of a new bath and thus to obtain greater current efficiency, use lower current densities if desired, and yet to form a uniform adherent deposit from a non-poisonous bath. The new bath also has excellent throwing power and hence is especially well adapted to the plating of irregularly shaped articles. Further objects and advantages of this invention will appear from a consideration of the following description of the new bath and the manner of its use.

According to the discovery upon which this invention is predicated it appears that triethanolamine, and probably other similar compounds, form with metals complexions somewhat similar, but more advantageous, in their affect in plating baths to the corresponding cyanides. Baths containing these ions may be used with particular advantage in the electrodeposition of metals upon cathodes on which the metals will not satisfactorily plate from the common plating

45

50

55

solutions. Such baths are non-poisonous and plate satisfactorily throughout a wide range of current densities. Many of the metals may be plated from solutions containing triethanolamine or other equivalent compounds, so that it will be possible here only to mention a few metals and plating solutions as illustrative. It is to be understood, however, that the principle of the invention is of general application.

As one example, an aqueous bath was prepared of the following formula:

Copper sulfate (5H<sub>2</sub>O) 150 grams/liter  
Boric acid 30 grams/liter  
Triethanolamine 270 c. c./liter

This bath was compared with an aqueous cyanide bath consisting of:

Cuprous cyanide 22.5 grams/liter  
Sodium cyanide 34.0 grams/liter  
Sodium carbonate 15.0 grams/liter

The results with the solutions stirred during deposition and run at 30 amperes per square foot, 5 volts potential were as follows:

| Time in seconds | Copper deposited mg./sq. cm. |              |
|-----------------|------------------------------|--------------|
|                 | New bath                     | Cyanide bath |
| 10              | .68                          | .016         |
| 30              | 3.27                         | .138         |
| 50              | 5.69                         | .220         |
| 70              | 7.74                         | .324         |
| 90              | 9.38                         | .428         |
| 120             | 11.91                        | .601         |

The deposit formed by the new process was bright, hard and copper colored. It was found preferable to use copper anodes to keep the solution supplied with the metal.

A modification of this bath that has proved particularly advantageous because of the high current efficiency that may be obtained therewith and because the deposit therefrom is especially satisfactory as a "strike" plate upon which further quantities of metal may be deposited has the following formula:

Copper sulfate (5H<sub>2</sub>O) 16 grams/liter  
Sodium oxalate 10 grams/liter  
Triethanolamine 22 c. c./liter

The solution so formed is light blue and does not plate on iron by contact. A current density of 3.6 amperes per square foot at 1.5 to 2.5 volts gives a bright plate on steel which will hold copper from the ordinary copper sulfate bath. Below are figures showing three test depositions under these conditions. They may be compared with the figures given above, but it should be remembered that the current density here is only about one-eighth of that used in obtaining those figures.

| Time in seconds | Copper deposited mg./sq. cm. |      |      |
|-----------------|------------------------------|------|------|
|                 | 1                            | 2    | 3    |
| 10              | .22                          | .06  |      |
| 20              |                              |      | .34  |
| 30              | .39                          | .36  |      |
| 50              | .74                          |      | .68  |
| 60              |                              | .76  |      |
| 70              | .91                          |      | .85  |
| 90              |                              | 1.05 |      |
| 120             | 1.44                         | 1.36 | 1.35 |

All deposits of 50 seconds or over from this bath were capable of holding a plate from an acid sulfate bath and deposits of 70 seconds or over were particularly well suited to this purpose.

As another example of the general principles or the invention the plating of nickel on zinc may be mentioned. Nickel will not ordinarily form an adherent deposit on zinc. However, good deposits on zinc can be obtained by the use of any one of several solutions containing a nickel salt and triethanolamine. The following solutions, which have been tried and found satisfactory may be cited as illustrative. Good throwing power is a characteristic of the solutions so that the deposit is smooth and uniform even though the cathode is irregularly shaped.

Nickel ammonium sulfate 120 grams/liter  
Triethanolamine 200 c. c./liter  
Water Remainder 20

(Boric acid may be added in small amounts but seems to have no appreciable effect.)

Temperature 20-25° C.  
Current density 5.83-23.57 amp./sq. dm. 25

Nickel ammonium sulfate 70 grams/liter  
Triethanolamine 100 c. c./liter  
Current density 21.6 amp./sq. dm.

Nickel ammonium sulfate 82.5 grams/liter 30

Triethanolamine 176 c. c./liter  
Current density 20-26 amp./sq. dm.

Nickel chloride (6H<sub>2</sub>O) 72.6 grams/liter  
Triethanolamine 48.4 c. c./liter  
Current density 18.28 amp./sq. dm. 35

Still further examples are furnished by the following aqueous solutions used for plating zinc, cobalt and cadmium respectively on copper, or other metals:

Zinc sulfate (7H<sub>2</sub>O) 75 grams/liter  
Triethanolamine 25 c. c./liter

White precipitate filtered out before use.

Cobaltus sulfate 75 grams/liter 45  
Triethanolamine 125 c. c./liter  
Current density 17 amps./sq. dm.

Cobaltous nitrate (6H<sub>2</sub>O) 75 grams/liter  
Triethanolamine 50 c. c./liter  
Current density 25 amps./sq. dm. 50

Cobaltous sulfate (6H<sub>2</sub>O) 75 grams/liter  
Triethanolamine 125 c. c./liter  
Current density 11 amps./sq. dm.

Plates well on zinc. 55

Cadmium sulfate 75 grams/liter  
Triethanolamine 25 c. c./liter

White precipitate filtered out before use.

Cadmium nitrate (4H<sub>2</sub>O) 75 grams/liter  
Triethanolamine 25 c. c./liter  
Current density 11 to 22 amps./sq. dm. 60

White precipitate filtered out before use.

While the invention has been described specifically by examples using triethanolamine in specific formulas in order to give a concrete understanding thereof, it is to be understood that the basic invention is not so limited but that other similar compounds may be substituted for the triethanolamine although triethanolamine is particularly effective and is for that reason definitely the preferred compound. Also, the formulas of the baths may be altered or new formulas devised and other metals than those mentioned may be plated and other metals may 75

receive the deposit. Also, although the invention is most advantageously used where the metal will not plate in an ordinary acid bath it may be used even though the metal will so plate when for any other reason it may be desired to plate the metal from the new type of solution.

As an example of the compounds that may replace triethanolamine in the practice of this invention di- and mono-ethanolamine may be mentioned and the use of other hydroxy alkyl amines and their substitution products and homologues particularly those having properties similar to triethanolamine are also contemplated. Other changes may be made to adapt the principles of this invention to various technical situations all within the skill of the chemist and the broadest scope of this invention.

We claim:

1. A method of electroplating that comprises contacting the object to be plated with a solution containing the metal to be deposited and an ethanolamine, and passing an electric current through said solution and object to deposit the metal thereon.
2. A method of electroplating that comprises contacting the object to be plated with a solution containing the metal to be deposited and an alkyloamine and passing an electric current through said solution and object to deposit the metal thereon.
3. A method of electroplating that comprises contacting the object to be plated with a solution containing the metal to be deposited and a trialkyloamine and passing an electric current through said solution and object to deposit the metal thereon.
4. A method of electroplating that comprises contacting the object to be plated with a solution containing the metal to be deposited and triethanolamine and passing an electric current through said solution and object to deposit the metal thereon.
5. A method of electroplating that comprises contacting the object to be plated with a solution containing the metal to be deposited, an oxalate

and an alkyloamine and passing an electric current through said solution and object to deposit the metal thereon.

6. A method of electrodepositing copper that comprises contacting the object to be plated with a solution containing copper and an alkyloamine, and passing an electric current through the solution and object to deposit the copper thereon.

7. A method of electrodepositing copper that comprises contacting the object to be plated with a solution containing around 150 grams per liter of copper sulfate and around 270 c. c. per liter of triethanolamine, and passing an electric current through the solution and object to deposit the copper thereon.

8. A method of electrodepositing copper that comprises contacting the object to be plated with a solution containing around 16 grams per liter of copper sulfate, around 10 grams per liter of sodium oxalate and around 22 c. c. per liter of triethanolamine, and passing an electric current through the solution and object to deposit the copper thereon.

9. A method of electrodepositing copper on iron that comprises contacting the iron with a solution containing copper, an oxalate and triethanolamine and passing an electric current through the solution and iron to deposit copper on the iron.

10. A method of electroplating that comprises contacting a zinc object to be plated with a solution containing nickel ammonium sulfate and around 100 to 200 c. c. per liter of triethanolamine and passing an electric current through said solution and object to deposit the nickel thereon.

11. A method of electroplating zinc that comprises contacting the object to be plated with a solution containing zinc and triethanolamine, and passing an electric current through the solution and object to deposit the zinc thereon.

12. A method of electroplating that comprises contacting a zinc object with a solution containing nickel and triethanolamine and passing an electric current through the solution to deposit the nickel thereon.

CHARLES JOSEPH BROCKMAN.